

## UNITED STATES PATENT OFFICE

2,206,090

WATERPROOFING COMPOSITION AND  
SIMILAR EMULSIONJohn E. Haggenmacher, Cranston, R. I., assignor  
to Warwick Chemical Co., West Warwick, R. I.,  
a corporation of Rhode IslandNo Drawing. Application May 17, 1937,  
Serial No. 143,119

13 Claims. (Cl. 134—15)

The present invention relates to improvements in emulsions and methods of making the same, and particularly relates to an improved waterproofing emulsion.

8 In the United States Patents 2,015,864 and 2,015,865 there are disclosed positively charged emulsions containing water insoluble materials, such as waxes, fats, oils, and so forth in disperse phase, which disperse phase is positively charged 10 and maintained by protective colloids and/or emulsifying agents.

15 It is among the objects of the present invention to provide improved emulsions and methods of making the same particularly designed for waterproofing purpose in which the disperse phase will have high stability in concentrated or diluted form under varying atmospheric conditions and upon storage.

20 Another object is to provide an improved waterproofing emulsion which will much more effectively treat fabrics, paper, cloth, furs and other materials to give them waterproof properties and which will be of high efficiency even in low concentrations.

25 Another object is to prepare an improved emulsion, particularly designed for waterproofing purposes, which will give a waterproofing of particularly high effectiveness, and which is devoid of foaming characteristics and will not tend 25 to form bubbles upon fabric or other materials and which, furthermore, will insure a uniform effect upon the fabrics without spotting or staining.

30 Another object is to provide an improved emulsion of the character described, having an increased surface tension and particularly designed for waterproofing purposes which will be devoid of complex organic protective colloidal materials such as glue, gelatine, casein, albumin, gums, 35 starches and so forth, which might tend to degrade or disintegrate or become modified upon standing, particularly in acidic environment.

Other objects will be obvious or will appear during the course of the following specification.

40 It has now been found that particularly stable emulsions, suitable for waterproofing purposes and containing an oil, wax or fat, or similar water-repellant materials, may be prepared by combining certain types of basic aliphatic compounds with these waxes, oils or fats and a positive 45 charging material such as a bivalent or trivalent metallic salt of a weak acid.

45 Among the preferred compounds which may be utilized are those formed by the combination of an aliphatic amine and a high molecular weight aliphatic compound, preferably containing more than eight carbon atoms, the preferred 55 compounds containing between 14 to 28 carbon atoms.

50 Among the preferred compounds, which may

be utilized are alcohols, ketones, acids, and esters containing one or more amido or amino groups, one or more sulphate or sulphonate groups and one or more of the following radicals, namely, 5 stearyl, abietyl, oleyl, linoleyl, ricinoleyl, ceryl, cetyl, myricyl, palmityl, dodecyl, octadecyl and so forth.

It has been also found satisfactory in some cases to utilize acids derived by the splitting of various vegetable or animal oils, fats and 10 waxes, such as the fatty acids which may be obtained by splitting or hydrolysis of the following oily materials, namely, olive oil, menhaden oil, palm oil, mustard seed oil, pea seed oil, cocoanut oil, cottonseed oil, rape seed oil, castor oil, 15 neat's-foot oil, peanut oil, lard oil, tallow oil, elaine oil, corn oil, sperm oil, fish oil, and/or cod oil or mixtures thereof.

These oils, or fatty acids, alcohols, ketones or 20 aldehydes containing about the same number of carbon atoms may also serve as the waterproofing materials.

Among the preferred fatty or aliphatic acid materials which may be employed are stearic acid, oleic acid, palmitic acid, linoleic acid, linolenic acid, ricinoleic acid, lauric acid, myristic acid, abietic acid, and so forth.

These acids are preferably combined with organic amino compounds preferably of an aliphatic nature which amino compounds may also 30 be hydroxylated or otherwise substituted.

Among the preferred amino compounds are those containing from two to ten carbon atoms and from one to five amino groups.

Among the compounds which may be preferred 35 are diethylene-triamine, triamino-propane, diamino-ethane, triaminopentane, mono- di- or triethanolamine, diamino-propanol, other mono- or poly-amino-alkanes, imino- or alkylamino alkanes, alkenes and alkynes, which may be also 40 substituted by groups, such as the —NO group, the —NO<sub>2</sub> group and so forth.

These amines may first be combined with the acids to form the ammonium salts or esters following which the combination may be dehydrated 45 with removal of water to form an amido combination.

These combinations are referred to in the specification and claims as "amido fatty acids" or as 50 "fatty acid amides."

However, if desired, the amino compound or compounds may be substituted directly in the aliphatic chain, whether the aliphatic chain be that of a fatty alcohol, ketone, aldehyde or acid and 55 this amino group may be combined with a low molecular weight acid followed by amidization.

In all of these cases the esters of the fatty acids or alcohols may be employed as may also their sulphonates where the sulphonic groups are at- 60

tached to the aliphatic chain or the sulphate-esters may be utilized.

According to one preferred method of carrying out the present invention, the amido compound is prepared by heating together the poly-amino alkane and the fatty acid which is to be combined with said amino compound.

Either one or both of these compounds may contain an aliphatic chain containing between 8 to 24 carbon atoms and these compounds are preferably reacted together in the proportions of 1 mol of the alkane to 1 mol of the acid although higher ratios of amines to acids are readily possible.

15 The mixture of the amine and acid is preferably heated up to a temperature above 150° C. until foaming subsides and until some or nearly all of the amino combination has been transformed into an amido combination.

20 The relative proportions of amido to amino groups may be widely varied depending upon the exact utilization of the compound.

To give one specific example, 1 mol of diethylene triamine or 103 grams thereof are added to 1 mol of molten or melted stearic acid or 284 grams thereof.

25 The heating and stirring together of the mixture is continued from 15 to 30 minutes with an optimum of about 20 minutes until the temperature reaches about 180 to 190° C.

Water will be liberated as a result of the amido formation and the end of the action will be apparent when the foaming subsides. After cooling, an amido stearyl diethylene amine is obtained.

If desired, the corresponding weights of palmitic, oleic, abietic or other fatty acids may be employed.

The resultant material is particularly designed as an emulsifying agent or as an emulsion stabilizer and the proportion of acid to amine may be varied depending upon the utilization.

If the material is to be utilized for emulsification of vegetable waxes, it is desirable to utilize from 1½ to 3 mols of amine of each mol of fatty acid.

Where the emulsifier is intended for the emulsification of mineral waxes, such as paraffin, the ratio of amine to fatty acid may be between 1 mol of the former to 1 to 3 mols of the latter.

This emulsifying agent may be incorporated in relatively small amounts with positively charging materials and with water insoluble fats, oils and waxes.

Among the preferred positive charging materials are metallic salts which on heating will form insoluble oxides such as the salts of zinc, aluminum or other bivalent and trivalent metals having amphoteric properties, preferably in combinations with weak acids as for example, organic acids.

Among the salts which may be utilized are the acetates, the formates, the gluconates or even the hydroxides in certain instances.

Among the water insoluble materials which can be utilized are the various oils disclosed above, as possible sources of fatty acids or as raw materials for the manufacture of fatty alcohols.

There also may be utilized various fats and waxes such as paraffin, ozokerite, ceresin, beeswax, candelilla wax, carnauba wax, japan wax, montan wax, spermaceti, chlorinated naphthalene or Halowax, petrolatum or petroleum jelly, with or without a wax mineral oil, benzene or even fatty acids such as stearic acids or the vari-

ous fatty acids and alcohols which may be derived from the oils above mentioned.

Under some conditions, paraffin oil, asphalt, bituminous substances and caoutchouc, may be used, but these materials are generally not preferred.

It is also possible to use colloidal stabilizer materials, such as gelatine, glue, albumin, casein, starch, gum, dimethyl cellulose, protalic acid, carbohydrates and sulphite waste liquors, but it has been found generally preferable to omit these colloidal stabilizer agents from the emulsifying mixture.

In making the emulsion, the waxy or the fatty material may be mixed with a small amount, 15 say 10% of the emulsifying material or amido compound. Then, the positive charging material may be added with stirring.

Finally, water may be added preferably at a temperature above 100° F. until a uniform mixture is obtained. This mixture is preferably passed through a colloid mill to assure thorough homogenization and combination thereof.

To give a specific example, 88 grams of paraffin wax and 6 grams of amido stearyl diethylene amine are melted together, following which 150 grams of aluminum acetate and 156 grams of water are added at a temperature of 140° F. while the mixture is being continually stirred. Then, this mixture is passed through a colloid mill.

It has been found generally desirable in making these mixtures to include only the water insoluble material or wax, that is wax, oil or fat, the amido emulsifying agent and the positive charging material, such as aluminum acetate.

Generally, the amido aliphatic emulsifying agent may constitute between 1 to 20% with a preferred range of 5 to 15% of the water insoluble material. The positive charging material may be between one tenth the weight of the water insoluble material to equal the weight of such material.

As a general rule, this combination of water insoluble material, positive charging material and emulsifier are mixed with from ¼ to 3 times their weight of water, and this emulsion then is in condition to be shipped and stored.

In case of treating fabrics, furs, leather or paper with the emulsion, water may be added in sufficient amount until the water insoluble material constitutes less than 10% and preferably less than 5% of the final emulsion.

For example, from 1 to 10% of the concentrated emulsion may be added to a water bath or from 1 to 10 parts of the emulsion may be diluted with 100 parts of water.

Preferably, the final treating bath should contain between 0.1 and 5% of the water insoluble material, whether it be oil, fat or wax or combinations thereof.

When textiles such as fabrics and yarns, whether of artificial silk, natural silk, cellulose acetate, cotton, linen, wool, and so forth, are treated with this diluted emulsion, the fabrics are dipped in the bath and permitted to remain in the bath with or without agitation for a period of 5 minutes to 1 hour.

All of the emulsions according to the above description have positively charged disperse phases and when they are subjected to electrical currents the dispersed particles will tend to move to the cathode. These emulsions are all perfectly stable in the concentrated form in which they are prepared. The non-aqueous con-

tent of these concentrated emulsions average usually substantially above 15%.

These emulsions will remain unchanged even after they have been kept for days at temperatures of zero to 10° F. At high temperatures of about 100° F. for example, these emulsions will remain completely stable, as contrasted to the usual negatively charged emulsions which contain no aluminum salts or similar electrolytes. 10 These latter emulsions will be destroyed if they are allowed to stand for a length of time at this temperature. It is obvious therefore that one of the advantages of the present invention resides in the fact that the emulsions produced will remain in stable condition in summer or in winter over long periods of time. This is requisite in commercial practice since these emulsions may be held in storage or in transport for days or weeks and they should not have undergone any change 20 during this period.

In lieu of aluminum acetate, it is also possible to utilize aluminum formate, aluminum sulphate, alum, and so forth. It is, however, contemplated that the aluminum salt may in part or whole be replaced by other polyvalent salts, such as copper sulphate, lead acetate, ferric sulphate, thorium nitrate, as well as acids, such as sulphuric acid, hydrochloric acid, acetic acid, and formic acid. These aluminum salts, or other polyvalent salts, 25 or acids are preferably used in a quantity varying between 10 to 60% or more of the water insoluble colloidal material.

These metallic salts and acids are referred to in the claims as positive charging agents or materials.

Although the present invention is particularly applicable to the impregnation and especially the waterproofing of textile materials, it is also broadly applicable to the treatment of paper and 40 paper pulp, furs, leather and skins, and other materials.

Although the emulsion is preferably utilized for waterproofing textiles in the form of fibers or yarns, it may also be utilized for softening, sizing, 45 lustering and otherwise finishing materials or incorporating loading materials therein.

Although the amido stearyl diethylene amine is the preferred emulsifying agent, there may also be used or included sodium lauryl sulphate, 50 sodium dodecyl sulphate, sodium octadecyl sulphate, combinations of fatty acid chlorides with proteins and other amino and amido organic compounds, stearyl mono-glycol amide, sodium myristyl amido sulphate, oleyl methyl amino 55 ethane sulphonic acid sodium salt, the sodium salt of oleylmethyltauric acid, a monoglycol ester of stearic acid, triethanol amine monoleic acid ester, esters of palmitic acid and dibutylethanolamines, a cocoanut oil fatty acid monoethanol 60 amide, stearic acid monoethanolamide, oleic acid diethanol amid, condensation products of ethylene oxides with fatty acids and alkyl amines and fatty acids and alkylol amines and the various esters, amides and compounds sold under the 65 names "Avirol," "Gardinol" and "Igepon".

Glue and gelatine and other similar protective colloids are preferably omitted.

It has been found that the waterproofing treatment of the present application may also be conveniently combined with a formaldehyde treatment, which formaldehyde treatment may precede or follow the waterproofing treatment.

This formaldehyde treatment is particularly desirable when the fabric has been sized or contains a water soluble colloid such as gelatin, glue,

a gum resin, and so forth, which should be insolubilized and prevent it from swelling and absorbing water during the waterproofing treatment or subsequent thereto.

Such treatment with formaldehyde may take place in a solution containing one part of formalin and three to ten parts of water.

If desired, instead of formalin, it is possible to use formaldehyde compounds such as paraform, hexamethylene tetramine, oxymethylene, and so forth.

A most unusual feature of the present invention resides in the discovery that it is possible to use certain high molecular weight aliphatic basic nitrogen containing ester or amide compounds, 15 which are insoluble in water, but are soluble in waxes, oils and fats to give a stabilized positively charged waxy, oily or fatty aqueous emulsion. These compounds when deposited upon the fabric do not have any affinity for moisture as is true in the case of glue, gelatin, gums, starches or other similar protective colloids. They thus give a better waterproofing effect.

The preferred compounds have the formula



25

where R, R<sub>1</sub> and R<sub>2</sub> are aliphatic or alkyl radicals at least one of which contains between 12 to 28 carbon atoms, and if desired one or both R<sub>1</sub> or R<sub>2</sub> may be hydrogen. Instead of a —CO— linkage, 30 it is also possible to have a —SO<sub>2</sub>— linkage, but this is not as preferred.

The formulae of the preferred compounds are possibly:



35



40

where n is between 12 and 28 and n<sub>1</sub> is between 1 and 4.

It is to be understood that the invention is not intended to be restricted to any particular example, composition or proportions, or to any particular application, or to any specific manner of use or to any of various details thereof, herein described, as the same may be modified in various particulars or be applied in many varied relations without departing from the spirit and scope of the claimed invention, the practical embodiments herein described merely showing some of the various features entering into the application of the invention.

What is claimed is:

1. An acidic waterproofing emulsion containing a positively charged disperse phase including a water repellent water insoluble matter, a water soluble positively charging material selected from the group consisting of polyvalent metal salts of bivalent and trivalent metals having amphoteric properties and acids and an amide combination of a high molecular weight fatty acid containing from 14 to 28 carbon atoms and a relatively low molecular weight aliphatic amine having between 1 and 6 carbon atoms.

2. For use in a process of waterproofing negatively charged textile materials, a dilute aqueous bath containing a positively charged colloidally dispersed water insoluble material, an amide combination of a high molecular weight fatty acid containing from 14 to 28 carbon atoms and a relatively low molecular weight aliphatic amine having between 1 and 6 carbon atoms serving as an emulsifying agent and a soluble polyvalent

55

45

50

55

60

65

70

75

amphoteric metallic salt, said bath having been prepared by the addition of a relatively large quantity of water to a relatively small quantity of a concentrated emulsion containing said water insoluble material, said agent and said polyvalent salt.

3. For use in a process of waterproofing negatively charged textile materials, a mixture of a relatively large quantity of water and a relatively small quantity of a concentrated emulsion containing an amide combination of a high molecular weight fatty acid containing from 14 to 28 carbon atoms and a relatively low molecular weight aliphatic amine having between 1 and 6 carbon atoms, a water soluble salt of a polyvalent metal having amphoteric properties and a water-insoluble material, the disperse phase of said emulsion being positively charged and said textile absorbing said oppositely charged waterproofing material in the disperse phase from said bath by reason of its opposite electric charge.

4. For use in a process of waterproofing negatively charged textile materials, a bath containing a relatively large quantity of water and a relatively small quantity of a concentrated emulsion containing an amide combination of a high molecular weight fatty acid containing 14 to 28 carbon atoms and a relatively low molecular weight aliphatic amine having between 1 and 6 carbon atoms, a water soluble aluminum salt and a paraffin wax, the disperse phase of said emulsion being positively charged and said textile absorbing said oppositely charged waterproofing material in the disperse phase from said bath by reason of its opposite electric charge.

5. For use in a process of waterproofing negatively charged textile materials, a bath containing a relatively large quantity of water and a relatively small quantity of a concentrated emulsion containing a paraffin wax, aluminum acetate and an amide combination of a high molecular weight fatty acid containing from 14 to 28 carbon atoms and a relatively low molecular weight aliphatic amine having between 1 and 6 carbon atoms, the disperse phase of said emulsion being positively charged and said textile absorbing the waterproofing material in the disperse phase from said bath by reason of its opposite electric charge.

6. For use in a process of waterproofing negatively charged textile materials, a bath containing a relatively large quantity of water and a relatively small quantity of a concentrated emulsion containing an amide combination of a high molecular weight of fatty acid containing from 14 to 28 carbon atoms and a relatively low molecular weight aliphatic amine having between 1 and 6 carbon atoms, aluminum acetate, petroleum jelly and a wax, the disperse phase of said emulsion being positively charged and said textile absorbing said oppositely charged waterproofing material in the disperse phase from said bath by reason of its opposite electric charge.

7. For use in a process of waterproofing negatively charged textile materials, containing a relatively large quantity of water and a relatively small quantity of a concentrated emulsion containing aluminum sulphate, mineral oil, stearyl diethylene amine and stearic acid, the disperse phase of said emulsion being positively charged and said textile absorbing said oppositely charged waterproofing material in the disperse

phase from said bath by reason of its opposite electric charge.

8. For use in a process of waterproofing negatively charged textile materials, a bath containing 20 to 100 parts of water and 1 part of a concentrated emulsion, said emulsion consisting of an amide combination of a high molecular weight fatty acid containing 14 to 28 carbon atoms and a relatively low molecular weight aliphatic amine having between 1 and 6 carbon atoms, a water soluble salt of a polyvalent metal having amphoteric properties and a water-insoluble material, the disperse phase of said emulsion being positively charged and said textile absorbing said oppositely charged waterproofing material in the disperse phase from said bath by reason of its opposite electric charge.

9. For use in a process of waterproofing negatively charged textile materials, a bath containing 20 to 100 parts of water and 1 part of a concentrated emulsion, said emulsion consisting of a mixture of 100 parts of waxy material, 2 to 10 parts of amido stearyl diethylene amine, 150 to 400 parts of water and 10 to 50 parts of aluminum acetate, the disperse phase of said emulsion being positively charged and said textile absorbing said oppositely charged waterproofing material in the disperse phase from said bath by reason of its opposite electric charge.

10. For use in a process of waterproofing negatively charged textile materials, a bath containing 20 to 100 parts of water and 1 part of a concentrated emulsion, said emulsion consisting of 6 parts of an amide combination of a high molecular weight fatty acid containing from 14 to 28 carbon atoms and a relatively low molecular weight aliphatic amine having between 1 and 6 carbon atoms, 700 parts of water, 30 parts of aluminum formate and 88 parts of paraffin, the disperse phase of said emulsion being positively charged and said textile absorbing said oppositely charged waterproofing material in the disperse phase from said bath by reason of its opposite electric charge.

11. For use in a process of waterproofing textiles with diluted aqueous emulsions of water insoluble oil, waxy and fatty materials as the positively charged disperse phase, said textiles being negatively charged, a concentrated emulsion with a positively charged disperse phase having a solid content of at least 15%, said solid content including the positively charged disperse phase constituting at least 20 to 50% of the emulsion, a stearyl amide as an emulsifying agent in amount from 5 to 15% of the disperse phase and a water soluble salt of a polyvalent metal having amphoteric properties in an amount ranging from 25 to 75% of the disperse phase diluted with at least 20 to 100 parts by weight of water per part of emulsion to form the bath.

12. An acidic waterproofing emulsion containing a positively charged disperse phase including a wax, a water soluble amide combination of a high molecular weight fatty acid containing from 14 to 28 carbon atoms and a relatively low molecular weight aliphatic amine having between 1 and 6 carbon atoms and a positively charging water-soluble material.

13. An acidic waterproofing emulsion containing a positively charged disperse phase including a wax, a stearic acid alkylene amide and an aluminum salt.

JOHN E. HAGGENMACHER.